

Sept. 7, 1943.

J. F. ECKERT, JR

**2,328,968**

## ART OF EXAMINING QUARTZ

Filed July 1, 1942



Joseph F. Eckert, Jr.  
Inventor  
C. D. Buska

23

**Attorney**

## UNITED STATES PATENT OFFICE

2,328,968

## ART OF EXAMINING QUARTZ

Joseph F. Eckert, Jr., Philadelphia, Pa., assignor  
to Radio Corporation of America, a corporation  
of Delaware

Application July 1, 1942, Serial No. 449,363

5 Claims. (Cl. 88—14)

This invention relates to the art of examining quartz and has special reference to a new and improved method of determining the orientation of a quartz bar, cube, or other partly fabricated piece of natural quartz of the type possessing piezoelectric properties.

In the manufacture of piezoelectric elements the crystal blanks are usually sliced from a pre-fabricated bar, cube or other unfinished quartz piece which may have any one of several orientations with respect to the natural crystalline axes of the mother crystal from which it was derived. Ordinarily the bars are cut from the mother crystal with an orientation calculated to provide the maximum useful number of finished elements. By way of example, as disclosed in U. S. Patent 2,264,698 to Charles E. Johnson, when the mother crystal comprises a small quartz "candle," it is preferable first to cut the mother crystal into a bar having long sides parallel to the optic axis and to thereafter slice the semi-finished blanks from the said bar. On the other hand, when the mother crystal is of a diameter substantially greater than, say, 2½ inches, the more common practice is to employ a bar or a cube cut from a slab having top and bottom surfaces which lie in planes normal to the optic axis. In any event, it will be apparent that before the unfinished blanks can be sliced from the larger piece, the lapidary must know the orientation and other characteristics of that particular piece or specimen. Thus, he must know (a) the location of its optic axis, (b) the virtual location and direction of tilt of the major and/or minor apex faces of the mother crystal from which the specimen was cut, and (c) whether the quartz is of the "right hand" or of the "left hand" variety. He should also preferably be informed as to the polarity of the X-axes in the said piece of quartz.

All, or at least some, of this information must, of course have originally been available to the lapidary in order to have enabled him to cut the bar itself from the mother crystal. However, before cutting a bar into blanks it is standard practice to etch the bar (as with hydrofluoric acid) in order to detect "twining," and other defects which, if present, would necessitate discarding the bar. Obviously, the etching process obliterates any identifying marks which may have originally been placed upon the bar.

Accordingly, one of the objects of the present invention is to provide a convenient and accurate method of determining the orientation of

an etched bar, cube or other partly fabricated piece of natural quartz.

Another and related object of the invention is to provide an improved method of locating the optic axis of an etched piece of quartz, and one which in its practice also reveals (a) whether the said piece is formed of "right hand" or of "left hand" quartz, (b) the virtual location of the direction of tilt of the major and/or minor apex faces of the mother crystal from which the piece was cut, and (c) the polarity and approximate location of the terminals of the X-axes in said piece.

A further object of the present invention is to provide a simplified method of examining quartz, and one which in its practice obviates the use of messy oils and expensive equipment.

Other objects and advantages will be apparent and the invention itself will be best understood by reference to the following specification and to the accompanying drawing, wherein

Figure 1 is a view in elevation of a quartz bar to which the invention is applicable and showing in outline a side section of the mother crystal from which the said bar was derived,

Figure 2 is a similar view of a quartz bar of another typical orientation, and to which the invention is applicable,

Figure 3 is a partly diagrammatic side elevational view of an apparatus which may conveniently be employed in carrying the invention into effect,

Figures 4 to 7 inclusive show certain patterns of light which appear in the quartz bars of Figs. 1 and 2 when inspected with the apparatus of Fig. 3, and which will be referred to in the following specification.

The invention will be described in connection with a problem commonly encountered in the commercial production of piezoelectric crystal elements from oblong bars whose long sides are substantially parallel either to the Z axis or to a Y axis of the mother crystal. It will be apparent, however, as the description proceeds that the invention is likewise applicable to quartz pieces of other shapes and of other orientations.

Fig. 1 shows a bar Q having its long sides substantially parallel to a Y axis and which has been cut in accordance with a standard procedure from a relatively large mother crystal.

Fig. 2 shows a bar Q' which has been cut in accordance with the teachings of U. S. Patent 2,264,698 to Charles E. Johnson, with its long sides parallel to the optic (Z) axis of the mother crystal.

Let us assume that these bars Q and Q' have reached that stage in their manufacture whereat they have been etched on all sides (to reveal any flaws in their natural crystalline structure) and hence are free from any previously applied markings indicative of their orientation. In such a case, it is obvious that before the semi-finished piezoelectric crystal elements or blanks can be cut from the said bars, it will be necessary for the lapidary to know the orientation and crystalline structure of each bar.

A spot source of light is employed in carrying the invention into effect. As shown in Fig. 3, the light may comprise an ordinary electric lamp 1 employing, say, a 40 watt bulb 2 and with the light therefrom directed upon the quartz piece Q through a pinhole 3 in a masking plate 4. The mask 4 may conveniently comprise either a turntable or a fixed support upon which the specimen rests during its inspection. When, as in the instant case, the piece of quartz to be examined comprises an oblong bar, it may be laid on its side, without clamping pressure, upon the plate 4 so that the spot of light impinges upon its bottom long surface. If the piece comprises a cube, it may first rest upon any of its surfaces. In accordance with the invention each face of the quartz specimen is presented to the spot of light until one of them reveals to the observer (indicated in Fig. 3 by the eye 5) a light pattern P Fig. 4, P' Fig. 5 in the form of a parallelogram having short sides 6 and 8 which intersect the long sides 7 and 9 at an angle other than a right angle. It has been discovered that the long sides of the parallelogram comprise, or are in register with, the optic (Z) axis of the quartz. Thus, to provide a permanent indication of the location of the optic axis it is merely necessary to draw a line Z-Z (as with a pencil, crayon, or stylus, not shown) on the specimen parallel to the long sides of the said parallelogram.

In order to determine whether the quartz is of the "right hand" or of the "left hand" variety, the specimen should first be so oriented with respect to the observer that one of the long sides of the parallelogram is to his right and the other to his left, as shown by way of example in Fig. 4. (In Fig. 5 wherein the optic axis Z-Z is parallel to the long sides of the specimen, the observer may either shift his position, or he may move the specimen 90° either in the clockwise or counter-clockwise direction). With the specimen in the desired position the long right side 9 of the parallelogram is used as a reference line. It is then necessary to note whether the acute (N. B., as distinguished from "obtuse") angle 6 formed by the intersection of this reference line 9 with one of the short sides (6 or 8) of the parallelogram P lies adjacent to the "top" or to the "bottom" of said parallelogram. If the said acute angle is at the top of the parallelogram, the specimen is constituted of "right hand" quartz; and if it is adjacent to the bottom of the parallelogram, it comprises "left hand" quartz. Thus the specimen Q, Fig. 4 is shown to be "right hand" quartz and the specimen Q' of Fig. 5 comprises "left hand" quartz. Since, as previously pointed out, any line drawn parallel to the long sides of the light pattern comprises the optic axis of the quartz it is obvious that the line 9 when suitably marked may be utilized as the reference optic axis, in which case the other line Z-Z is superfluous, and need not be marked upon the specimen.

The short sides 6 and 8 of the light pattern reveal the virtual location and direction of tilt, with respect to the optic axis, of a major apex face of the mother crystal from which the specimen was derived. Accordingly, when this information is required to be known the specimen may be permanently marked with such a line, as indicated at M-M. In some cases, as where the etching is unduly shallow, or unduly deep, the said short sides of the parallelogram may not provide an exact indication of the location of a major apex face of the mother crystal. This, however, is of no especial moment since (a) the indication of the direction of slope is the important thing and (b) the exact angle formed by the intersection of a major or a minor face with the optic axis is known to be approximately 38° 14' and, since the direction of slope has been indicated, it is a relatively simple matter to check the accuracy of the indication provided by the said short sides of the light pattern.

The present invention does not lend itself readily to the accurate location of the X and Y axes of a quartz specimen. However, it may here be noted that the electrically positive (+) terminal of the X-axes will always lie adjacent to the surface of the specimen upon which the above described parallelogram light pattern appears.

Figs. 6 and 7 show the light patterns which are obtained by directing the spot of light upon the (positive) surface of the crystal upon which the "closed" parallelograms of Figs. 4 and 5 appear. It will be observed that the principal difference between the patterns shown in Figs. 4 and 6, and in Figs. 5 and 7, resides in the fact that in Figs. 6 and 7 the edges of the light pattern extend beyond the boundaries of the parallelogram. Further, in practice, the latter patterns may not be as clearly defined as the ones shown in Figs. 4 and 5. Accordingly, in practicing the present invention, it is preferable to seek the "closed" light patterns of Figs. 4 and 5 rather than the "openwork" or "criss-cross" patterns of Figs. 6 and 7, though either may be utilized. If these latter patterns are employed it is, of course, necessary to bear in mind that a line N-N drawn parallel to the short sides 6 and 8 of the light pattern will show the direction of slope of a minor instead of a major, apex face of the mother crystal.

It will now be apparent that the present invention comprises a simple, inexpensive and trouble-free method of examining rapidly a quartz specimen to determine (a) the location of its optic axis (b) the virtual location and direction of tilt of the major and minor apex faces of the mother crystal from which the specimen was derived, (c) whether the quartz is of the "right hand" or "left hand" variety, and (d) the location of the positive and negative faces of the specimen.

What is claimed is:

1. Method of locating the optic axis of an etched piece of quartz, said method comprising directing a spot of light upon different surface areas of said quartz piece until a light pattern in the form of a parallelogram having long and short sides which intersect at an angle other than a right angle is revealed to an observer looking into said piece from the opposite side thereof, marking on said piece a line drawn parallel to the long sides of said parallelogram, and designating the said line as the optic axis.

2. Method of locating the optic axis and of determining the polarity of the surfaces of an

etched piece of quartz, said method comprising directing a spot of light upon different surfaces of said quartz piece until a light pattern in the form of a parallelogram having long and short sides which intersect at an angle other than a right angle is revealed to an observer looking into said piece from the opposite side thereof, marking the side of the quartz upon which said pattern appears as the electrically positive (+) side of the said piece, marking said piece with a line drawn parallel to the long sides of said parallelogram and designating the said line as the optic axis of said quartz.

3. Method of inspecting an etched piece of quartz to locate the optic axis, and the virtual location and direction of tilt, with respect to the optic axis, of a major apex face of the mother crystal from which said piece was derived, said method comprising directing a spot of light upon different surface areas of said quartz piece until a light pattern in the form of a parallelogram having short sides which intersect the long sides at an angle other than a right angle is revealed to an observer looking into said piece from the opposite side thereof, marking on said surface a line parallel to the long sides, and a second line parallel to the short sides of said parallelogram, designating said first mentioned line as the optic axis of said piece, and designating said second mentioned line as a side edge of a major apex

face of the mother crystal from which said quartz piece was derived.

4. Method of examining an etched piece of quartz to determine whether said quartz is of the "right hand" or of the "left hand" variety, said method comprising directing a spot of light upon various surface areas of said quartz piece until a light pattern in the form of a parallelogram having short sides which intersect the long sides at an angle other than a right angle is revealed to an observer looking into the piece from the opposite side thereof, orienting said quartz piece with respect to the observer until one of said long sides of said parallelogram is to the right and the other long side of said parallelogram is to the left of said observer, designating said long right side of said parallelogram as a reference line, and then marking said quartz to be (a) of the "right hand" variety or (b) of the "left hand" variety as determined by whether the acute angle formed by the intersection of said reference line with one of said short sides of said parallelogram lies adjacent to (a) the top or (b) to the bottom of said parallelogram.

5. Method of examining quartz in accordance with the preceding claim and including the additional step of designating said reference line as the optic (Z) axis of said quartz piece.